

## UNITED STATES PATENT OFFICE

2,035,414

## ALLOYS

Richard A. Wilkins, Rome, N. Y., assignor to  
 Revere Copper and Brass Incorporated, Rome,  
 N. Y., a corporation of Maryland

No Drawing. Application March 2, 1935,  
 Serial No. 9,110

## 6 Claims. (Cl. 75—1)

My invention relates to alloys.

Applicant has found that ternary copper-silicon-tin alloys with a high copper content and the silicon and tin within certain ranges and proportions possess a high resistance to corrosion, a high tensile strength, and relatively high ductility or elongation in both the fully annealed and cold worked conditions, and that they may be heat treated when cold worked markedly to increase their yield point without reduction or marked change in tensile strength, ductility and hardness.

It has been found that if iron is added to these alloys the hardness may be controlled both by varying the amount of iron and by heat treatment of the alloy without materially decreasing the resistance to corrosion or other properties of the alloy except a slight increase in tensile strength at the expense of a slight decrease in ductility.

Preferably the amount of iron is such in relation to the amount of silicon as to cause all the iron to be in the form of iron silicide, thus avoiding the presence of free iron which otherwise would be present due to the insolubility of the iron in the copper-base. Any deleterious effect on the corrosion resistance of the alloy due to the presence of iron silicide and minute quantities of free iron is more than offset by the tin. The iron silicide it has been found apparently dissolves in the fully annealed alloy, but precipitates in the heat treated alloy to form needle-like crystals which act to lock together the glide planes of the crystals which act to lock together planes of the crystals of the basic alloy. Thus in the fully annealed alloy the hardness is not materially affected by the addition of iron to the basic alloy, but in the heat treated alloy the addition of iron secures a noticeable hardening effect.

In the improved alloy, although the preferred range of silicon is approximately 2.75 to 3.5%, below which range the tensile strength and yield point increasingly decrease and above which range the alloy becomes increasingly difficult to cold work, the silicon in many instances may be as low as 2% and still an alloy be secured which has the desired properties.

The alloy in respect to many of its properties is rather sensitive to iron, and ordinarily the latter should be maintained between approximately 0.1 and 0.6% so as not deleteriously to affect the properties of the alloy. A preferred value of 0.25% iron ordinarily gives excellent results.

The preferred range of tin for the above mentioned preferred range of silicon is 0.25 to 0.5%, but by maintaining a proper relation between the tin and silicon the amount of tin in some instances may be materially increased. As little as 0.25% tin may be present for all values of silicon from 2 to 3.5%, but to maintain the alloy hot workable within this range of silicon the tin should not exceed approximately 2% for 3% silicon and a progressively decreasing value as the silicon is increased or decreased above or below 3%. Approximately, with any value of silicon less than 3%, the amount of tin should not exceed a value which decreases linearly from 2% at 3% silicon at the rate of about  $\frac{1}{4}\%$  for 1% decrease in silicon from 3%, that is to say, no more than about 1.75% tin may be employed with 2% silicon. Approximately, with any value of silicon more than 3%, the amount of tin should not exceed a value which decreases linearly from 2% at 3% silicon at the rate of about  $\frac{5}{8}\%$  for 1% increase in silicon from 3%, that is to say, no more than about 1.7% tin should be employed with 3.5% silicon.

The alloy may be fully annealed by heating it to about 1200 to 1300° F., and within the preferred range of 2.75 to 3.5% silicon, 0.25 to 0.5% tin, and 0.25% iron, all the alloys will have a tensile strength of at least approximately 60,000 pounds per square inch and an elongation of at least approximately 60% in two inches. These alloys may be cold drawn into rods having a tensile strength of at least approximately 125,000 pounds per square inch and an elongation of at least approximately 9% in two inches, and may be cold rolled into sheets having a tensile strength of at least approximately 115,000 pounds per square inch and an elongation of at least approximately 4% in two inches. In general all the alloys within the larger ranges of constituents above specified have a tensile strength of at least 58,000 pounds per square inch and an elongation of at least approximately 60% in two inches when in the fully annealed condition, and are capable of being cold drawn into rods having a tensile strength of at least 120,000 pounds per square inch and an elongation of at least approximately 9% in two inches, and are capable of being cold rolled into sheets having a tensile strength of at least 110,000 pounds per square inch and an elongation of at least approximately 4% in two inches.

When fully annealed the alloys are capable of at least 50% reduction by cold rolling or cold drawing without again annealing them. This enables them readily to be cold worked into arti-

- cles. By heating the cold worked articles to 500 to 600° F. for 30 to 90 minutes and cooling them in air at room temperature the yield point and hardness of the alloy will be markedly increased 5 without any material change in the tensile strength and elongation. It will be observed that this heat treatment is performed at temperatures below the full annealing temperatures, or, in other words, is performed at temperatures below the recrystallization temperatures of the copper-silicon-tin solution, although performed at the temperatures at which dissolved iron silicide 10 will precipitate as has hereinbefore been referred to.
- 15 The alloys described, besides being capable of hot rolling and drawing enabling mill products economically to be fabricated of them, and capable of being cold rolled and drawn and otherwise cold worked, present superior alloys for welding 15 purposes.
- 20 It will be understood that small amounts of metals other than those herein specified may be added to the alloys for imparting special characteristics when these metals do not destroy such 25 valuable properties of the alloy as it may be desired to retain.
- I claim:
1. Copper base alloys capable of being worked both hot and cold containing copper, silicon, tin 30 and iron within the following approximate ranges

and proportions: silicon 2 to 3.5%, tin 0.25 to 2%, iron 0.1 to 0.6%, balance substantially all copper, the minimum amount of tin being 0.25% for all values of silicon, the maximum amount of tin varying between 1.75 and 2% directly and linearly with the amount of silicon when the latter is between 2 and 3% and varying between 1.7 and 2% inversely and linearly with the amount of silicon when the latter is between 3 and 3.5%; the alloys being of relatively high tensile strength 10 and ductility in both the fully annealed and cold worked conditions, and when cold worked from the fully annealed condition being capable of being heat treated for markedly increasing both the yield point and hardness with but relatively 15 small change in the tensile strength and ductility.

2. The alloys according to claim 1 having approximately 0.25% iron.

3. The alloys according to claim 1 having approximately 2.75 to 3.5% silicon.

4. The alloys according to claim 1 having, approximately, 2.75 to 3.5% silicon and 0.25 to 0.5% tin.

5. The alloys according to claim 1 having, approximately, 2.75 to 3.5% silicon and 0.25% iron.

6. The alloys according to claim 1 having, approximately, 2.75 to 3.5% silicon, 0.25 to 0.5% tin, and 0.25% iron.

RICHARD A. WILKINS. 30

#### CERTIFICATE OF CORRECTION.

Patent No. 2,035,414.

March 24, 1936.

RICHARD A. WILKINS.

It is hereby certified that error appears in the printed specification of the above numbered patent requiring correction as follows: Page 1, first column, line 14, for "harness" read hardness; and lines 34 and 35, strike out the words "which act to lock together planes of the crystals"; and that the said Letters Patent should be read with these corrections therein that the same may conform to the record of the case in the Patent Office.

Signed and sealed this 28th day of April, A. D. 1936.

Leslie Frazer

Acting Commissioner of Patents.

(Seal)

- cles. By heating the cold worked articles to 500 to 600° F. for 30 to 90 minutes and cooling them in air at room temperature the yield point and hardness of the alloy will be markedly increased 5 without any material change in the tensile strength and elongation. It will be observed that this heat treatment is performed at temperatures below the full annealing temperatures, or, in other words, is performed at temperatures below the recrystallization temperatures of the copper-silicon-tin solution, although performed at the temperatures at which dissolved iron silicide 10 will precipitate as has hereinbefore been referred to.
- 15 The alloys described, besides being capable of hot rolling and drawing enabling mill products economically to be fabricated of them, and capable of being cold rolled and drawn and otherwise cold worked, present superior alloys for welding 15 purposes.
- 20 It will be understood that small amounts of metals other than those herein specified may be added to the alloys for imparting special characteristics when these metals do not destroy such 25 valuable properties of the alloy as it may be desired to retain.
- I claim:
1. Copper base alloys capable of being worked both hot and cold containing copper, silicon, tin 30 and iron within the following approximate ranges

and proportions: silicon 2 to 3.5%, tin 0.25 to 2%, iron 0.1 to 0.6%, balance substantially all copper, the minimum amount of tin being 0.25% for all values of silicon, the maximum amount of tin varying between 1.75 and 2% directly and linearly with the amount of silicon when the latter is between 2 and 3% and varying between 1.7 and 2% inversely and linearly with the amount of silicon when the latter is between 3 and 3.5%; the alloys being of relatively high tensile strength 10 and ductility in both the fully annealed and cold worked conditions, and when cold worked from the fully annealed condition being capable of being heat treated for markedly increasing both the yield point and hardness with but relatively 15 small change in the tensile strength and ductility.

2. The alloys according to claim 1 having approximately 0.25% iron.

3. The alloys according to claim 1 having approximately 2.75 to 3.5% silicon.

4. The alloys according to claim 1 having, approximately, 2.75 to 3.5% silicon and 0.25 to 0.5% tin.

5. The alloys according to claim 1 having, approximately, 2.75 to 3.5% silicon and 0.25% iron.

6. The alloys according to claim 1 having, approximately, 2.75 to 3.5% silicon, 0.25 to 0.5% tin, and 0.25% iron.

RICHARD A. WILKINS. 30

#### CERTIFICATE OF CORRECTION.

Patent No. 2,035,414.

March 24, 1936.

RICHARD A. WILKINS.

It is hereby certified that error appears in the printed specification of the above numbered patent requiring correction as follows: Page 1, first column, line 14, for "harness" read hardness; and lines 34 and 35, strike out the words "which act to lock together planes of the crystals"; and that the said Letters Patent should be read with these corrections therein that the same may conform to the record of the case in the Patent Office.

Signed and sealed this 28th day of April, A. D. 1936.

Leslie Frazer

Acting Commissioner of Patents.

(Seal)

CERTIFICATE OF CORRECTION.

Patent No. 2,035,414.

March 24, 1936.

RICHARD A. WILKINS.

It is hereby certified that error appears in the printed specification of the above numbered patent requiring correction as follows: Page 1, first column, line 14, for "harness" read hardness; and lines 34 and 35, strike out the words "which act to lock together planes of the crystals"; and that the said Letters Patent should be read with these corrections therein that the same may conform to the record of the case in the Patent Office.

Signed and sealed this 28th day of April, A. D. 1936.

Leslie Frazer

(Seal)

Acting Commissioner of Patents.